

Nov. 15, 1949

F. E. BUCHAN

2,487,788

PROCESSING OIL SHALE

Filed Sept. 5, 1945



Inventor:  
Frederick E. Buchan  
By Donald G. Welsh  
Attorney

Patented Nov. 15, 1949

2,487,788

# UNITED STATES PATENT OFFICE

2,487,788

## PROCESSING OIL SHALE

Frederick E. Buchan, Washington, D. C., assignor  
to the United States of America as represented  
by the Secretary of the Interior

Application September 5, 1945, Serial No. 614,588

6 Claims. (Cl. 196—56)

(Granted under the act of March 3, 1883, as  
amended April 30, 1928; 370 O. G. 757)

1

The invention herein described and claimed  
may be manufactured and used by or for the Gov-  
ernment of the United States of America for gov-  
ernmental purposes without the payment of any  
royalties thereon or therefor.

This invention relates to the recovery of hydro-  
carbon liquids and/or gases from carbonaceous  
mineral materials, more particularly to the pro-  
duction of high quality liquid fuel fractions from  
kerogen rocks.

It is an object of the invention to increase the  
yield of useful products from kerogen rocks, es-  
pecially oil shales such as occur in the United  
States. Another object of the invention is the  
recovery of crude liquid hydrocarbons that may  
be further processed satisfactorily either by con-  
ventional refining operations or, at the most, with  
only minor modification thereof. A further ob-  
ject is the provision of an improved heating meth-  
od whereby the percentage recovery as a liquid  
of the organic matter initially present in the rock  
is materially increased over prior methods, with-  
out excessive decomposition and consequent for-  
mation of carbon in the residual material. Other  
objects will be apparent or will appear herein-  
after.

Kerogen rocks are defined by Down and Himus  
(Classification of Oil Shales and Cannel Coals  
(1940)) as sedimentary rocks containing organic  
matter which, on destructive distillation, yield  
an oil equivalent to approximately 50 percent of  
the organic content. They occur in continuous  
seams scattered all over the world, and the west-  
ern deposits in the United States are particularly  
suitable for development, although large quanti-  
ties of lean oil shale occur in the Kentucky-In-  
diana area. A typical sample of Green River  
shale from Colorado according to Bradley (Geol.  
Survey Prof. Paper 168 (1931)) consists of kero-  
gen 46 percent, clay 21 percent, excess silica 10  
percent, and magnesium carbonate 9 percent.  
Kerogen itself, according to Brown (Shale Oil—  
R. N. McKee (1925)) is the material in Scottish  
shales, which, on destructive distillation, yields  
oil. It is neither petroleum nor bitumen, but an  
organic substance yielding petroleum and nitro-  
genous compounds upon pyrolytic conversion.

It has been the common practice for many  
years to distill destructively kerogen rocks, such  
as Scottish shale in large vertical retorts thereby  
decomposing the kerogen and recovering part of  
it in the form of oils resembling crude petroleum  
while a part of it is lost as fixed gases and residual  
carbon. However, the percentage recovery, as  
oil, of the organic matter present in the shale is  
low and this fact has led to the development of  
many types of retorts to improve the process. In  
spite of all these efforts, to date the total recov-  
ery of the kerogen in the shale remains relatively  
low, as some of it is always reduced to carbon and  
permanent gases, which have some usefulness but  
are not particularly useful as the crude oils.

5 In order to overcome this difficulty, it has been  
proposed to extract the kerogen from the shale  
with liquid solvents, and thereby increase the re-  
covery of crude oils and avoid the formation of  
excess carbon and permanent gases. Numerous  
patents have been granted covering the broad as-  
pects of this idea, but so far a successful process  
to compete with the established retort methods,  
has not been developed.

10 In my investigations of the broad problem of  
extractive recovery of organic matter in oil shales  
and other kerogen rocks, I have discovered the  
following pertinent facts:

15 1. Kerogen itself is not soluble in the usual liq-  
uid solvents and various fractions of shale oil and  
similar liquids, previously proposed for its ex-  
traction.

20 2. On heating at various temperatures for vary-  
ing periods of time, kerogen is converted to bitu-  
men, the percentage conversion increasing  
with the temperature and time of heating.

25 3. The resulting bitumen is soluble in certain  
fractions of shale oil, including the heavier frac-  
tions.

30 4. Prolonged contact of the extracted bitumen  
with the remaining shale results in cracking of  
the bitumen to yield various lower boiling frac-  
tions of liquid hydrocarbons, such as gas, gaso-  
line, fuel oil, etc., the extent of the cracking de-  
pending on the time of contact and temperature.

35 The correlation of temperature and time of di-  
gestion with respect to items 2 and 4 above in the  
batch treatment of a Colorado oil shale are sum-  
marized in the tables below:

| 40                |                        | Heating Time (Hours) |      |      |     |
|-------------------|------------------------|----------------------|------|------|-----|
|                   |                        | 0.5                  | 1.0  | 1.5  | 2.0 |
|                   | I. T=707° F. (375° C.) |                      |      |      |     |
| Kerogen converted | 6.9                    | 13.4                 | 19.4 | 25.0 |     |
| Gas               | 2.4                    | 4.9                  | 7.2  | 8.7  |     |
| Light Oils        | 0.6                    | 1.2                  | 1.7  | 2.2  |     |
| Heavy Oils        | 3.9                    | 7.3                  | 10.5 | 14.1 |     |
| Carbon            |                        |                      |      |      |     |

| 50                |      | II. T=752° F. (400° C.) |      |      |      |
|-------------------|------|-------------------------|------|------|------|
|                   |      | 22.1                    | 39.4 | 52.8 | 63.2 |
| Kerogen converted | 22.1 | 39.4                    | 52.8 | 63.2 |      |
| Gas               | 3.0  | 5.9                     | 8.5  | 10.9 |      |
| Light Oils        | 2.6  | 4.6                     | 6.2  | 7.9  |      |
| Heavy Oils        | 16.5 | 28.9                    | 38.1 | 44.5 |      |
| Carbon            | NH   | NH                      | (?)  | (?)  |      |

| 55                |       | III. T=797° F. (425° C.) |        |        |      |
|-------------------|-------|--------------------------|--------|--------|------|
|                   |       | 51.8                     | 76.8   | 88.8   | 96.0 |
| Kerogen converted | 51.8  | 76.8                     | 88.8   | 96.0   |      |
| Gas               | 4.7   | 9.0                      | 13.0   | 18.9   |      |
| Light Oils        | 6.2   | 11.0                     | 14.9   | 19.0   |      |
| Heavy Oils        | 34.9  | 44.8                     | 42.9   | 33.1   |      |
| Carbon            | (6.0) | (12.0)                   | (18.0) | (25.0) |      |

60 NOTE: Figures represent percentage by weight based on the kero-  
gen initially present in shale.

These data indicate that under the conditions

of these tests there is an optimum relation of time and temperature for the maximum conversion of kerogen to liquid fuels, such as gasoline and heavier oils, and a minimum conversion to gases and residual carbon. Obviously with other shales, the yields and products distribution may vary from those given above for like conditions, and the optimum conversion conditions for yields of liquid products may differ with shales of varying kerogen content.

Based on experimental evidence available at this time, my treating process may be considered as involving the following stages:

1. Initial heating of shale to a predetermined temperature and to drive off free moisture in the shale.

2. Conversion of kerogen of the shale to bitumen and some lighter products.

3. Cracking of bitumen and heavy oil to lighter products.

This theory is advanced merely by way of explanation and it will be understood that the description of my invention is not intended to be limited to any particular theory as to the mechanism of the reaction whereby kerogen of the shale is recovered as useful liquid products.

In a batch treatment, as described herein, by reason of lack of uniformity in the chemical composition and physical character of the charge, the heating rate and other factors, obviously these stages will not appear to be separate and distinct. Some conversion of kerogen to bitumen and cracking of bitumen and heavy oil may occur during the initial heating stage. Likewise there may be appreciable cracking of heavier products concurrently with the conversion of kerogen to bitumen in the second stage of the process. In general, however, each stage will be characterized by the predominant physical or chemical changes occurring at the time.

In my combined heating and extracting method for the recovery of shale oil, I have found that it is unnecessary to resort to fine grinding of the raw shale and that the process is effective if the shale is coarsely crushed to about one-half inch size.

A suitable procedure for realizing the desired optimum conditions for conversion of the kerogen of oil shale to useful liquid products is described in connection with the accompanying drawing.

A Colorado oil shale, crushed to approximately one-half inch size, is fed into a vertical reactor 1, which is preferably lagged to minimize heat loss. When the desired quantity of material has been placed in the reactor, a high boiling fraction of shale oil is withdrawn from tank 3 passing through valve controlled line 15 and pump 16 to heater 4. In heater 4, the heavy oil is heated to about 425° C. and passes to reactor 1 through line 10. The overflow from reactor 1 passes through line 7 to separator 2 where water vapor and lighter oils are separated and oils heavier than furnace oils are withdrawn through line 8 to heater 4 and back to reactor 1. Heavy oil over and above that required for the extractive treatment of the shale is accumulated in tank 3 and may be withdrawn from the system by line 20. The flow of heavy oil to tank 3 is controlled by closing valve 9 and opening valve 22.

Lighter products, including gases and water, removed from the circulating stream in separator 2, flow through line 12 to stripper 6. Gases are taken off overhead from stripper 6 through line

14, while the light liquid products flow out through line 13 for further treatment.

The gases taken off at 14 may be used as fuel in heater 4 or may be separated into various fractions as is well known in the refining art.

Fractions of intermediate boiling range, such as furnace oil, gas oil, and the like may be withdrawn in one or more side streams, as at 11, from separator 2.

For a maximum recovery of liquid fuels from Colorado oil shale, circulation of the heavy oil at about 425° C. is maintained for not in excess of one and one-half hours after the oil shale charge is brought to this temperature. Under these conditions, as shown in the above tables, approximately 90 percent of the kerogen is converted to extractable material, and at least 18 percent light oil and 42 percent heavy oils will be recovered. This is equivalent to a conversion of 60 percent of the total kerogen to liquid products, of which the major portion represents desirable liquid fuel fractions.

By operating at a lower temperature for a longer period of time, a higher proportion of the extracted bitumen may be recovered as useful liquid fuels, although there will be a corresponding decrease in kerogen conversion and the total amount of these liquid products recovered may be lower than when the conditions are as described in the foregoing example. From a two and one-half hour treatment at 400° C., the recovery of liquid products on the basis of kerogen converted (57/71)=80 percent as compared with (60/90)=67 percent under the higher temperature and shorter time conditions. Where an increased recovery of heavier oils is desirable such conditions obviously are indicated.

At the end of the treating period, circulation of the heavy oil through heater 4 is discontinued and valve 23 is closed. Liquid materials in reactor 1 are allowed to drain into surge tank 5 through line 18 by opening valve 24 and closing valve 19. Any oil remaining in or on the treated shale in reactor 1 may be recovered by displacement with steam or gases admitted through valve controlled line 21. The spent shale in reactor 1 is then discharged and the reactor is refilled with fresh oil shale. The contents of tank 5 are pumped through line 17 and heater 4 into reactor 1 by closing valve 24 opening valves 23 and 25 and starting pump 16. Additional oil to fill the reactor is drawn from tank 3 and the treating cycle is repeated.

For reasons of economy of operation, a plurality of reactors 1 may be employed with suitable connections to heater 4, surge tank 5 and separator 2, so that at the close of the treating cycle in one reactor, treatment of fresh shale may be continued in a second reactor. In this manner heavy oil and any material dissolved therein may be continuously circulated through heater 4, the shale charge in one of the reactors 1 and separator 2 back to the heater 4, without a substantial loss of process time in charging and discharging the reactors 1.

It is understood, of course, that my invention is not limited to the exact conditions and embodiments shown and described herein and that various other means and conditions may be employed within the scope of the appended claims.

I claim:

1. A process for the recovery of valuable liquid products from kerogen containing rock which comprises treating kerogen containing rock in coarsely crushed form with a hydrocarbon oil

maintained at a temperature within the range of about 375°-425° C. and for a period of time not in excess of two and one-half hours thereby converting a substantial portion of the kerogen of said rock to predominantly liquid products, miscible with said oil, removing fluids from contact with the treated rock and fractionating the thus separated fluids into fractions of desired boiling ranges.

2. A process as in claim 1 in which the hydrocarbon treating oil comprises a fraction of the heavy oils produced from kerogen containing rock, said fraction having an initial boiling point above 200° C.

3. A process as in claim 1 in which the treating period is between one and two hours.

4. A process as in claim 1 in which the yield of liquid products is equivalent to at least fifty percent of the kerogen initially present in the rock.

5. A process for increasing the percentage recovery of normally liquid hydrocarbons from the pyrolytic conversion of kerogenous materials which comprises subjecting kerogen containing solids in the form of coarsely crushed lumps to the action of a heavy hydrocarbon oil at a temperature within the range of from 375° C. to 425° C. for at least one hour and not substantially in excess of two hours, separating the thus treated solids from the said oil and liquid conversion products, distilling the separated effluent and recovering fractions of desired boiling ranges.

5

6. A process for the production of hydrocarbon oils from oil shales which comprises passing a shale oil fraction heavier than furnace oil in contact with shale in a conversion zone maintained within the range 375°-425° C., fractionating effluent from said reaction zone to separate lighter products and to recover a fraction heavier than furnace oil, heating said heavier fraction to the temperature of said conversion zone and returning said heated fraction to said conversion zone, circulation of said heavier fraction being continued for from one to two hours, whereby substantial conversion of kerogen to hydrocarbon oils is effected, separating the thus treated shale from further contact with said oil and conversion products and recovering fractions of desired boiling ranges from said oil and conversion products.

FREDERICK E. BUCHAN.

20

#### REFERENCES CITED

The following references are of record in the file of this patent:

#### UNITED STATES PATENTS

|    | Number     | Name          | Date           |
|----|------------|---------------|----------------|
| 25 | Re. 17,762 | Reeve I       | Aug. 5, 1930   |
|    | 1,327,572  | Ryan          | Jan. 6, 1920   |
|    | 1,467,758  | Day II        | Sept. 11, 1923 |
|    | 1,643,521  | Reeve II      | Sept. 27, 1927 |
| 30 | 1,778,515  | Hampton       | Oct. 14, 1930  |
|    | 1,833,155  | Danner et al. | Nov. 24, 1931  |
|    | 1,903,749  | Carter        | Apr. 11, 1933  |
|    | 2,397,432  | Records       | Mar. 26, 1946  |